

Patented Mar. 20, 1923.

1,449,154

## UNITED STATES PATENT OFFICE.

CALVIN SPENCER VIDEON, OF TOTTENVILLE, NEW YORK, ASSIGNOR TO THE S. S. WHITE DENTAL MANUFACTURING COMPANY, A CORPORATION OF PENNSYLVANIA.

### ALLOY.

No Drawing.

Application filed May 10, 1919. Serial No. 296,177.

To all whom it may concern:

Be it known that I, CALVIN SPENCER VIDEON, a citizen of the United States, and a resident of Tottenville, county of Richmond, 5 State of New York, have invented certain new and useful Improvements in Alloys, of which the following is a specification.

My invention relates particularly to that class of alloys that are composed principally 10 of precious metals and that will withstand the action of heat and of acids without detrimental effects, and is especially directed to alloys employed in the manufacture of retaining pins for artificial teeth.

15 The principal objects of my invention are to provide an alloy that may be employed in the manufacture of artificial teeth with an efficiency substantially equal to platinum and with materially less expense.

20 My invention comprehends an alloy that will withstand heat sufficient to fuse artificial teeth to the porcelain state, that will not oxidize, nor be affected by the acids contained in the fluids of the human mouth, and 25 that will withstand the strains to which a tooth may be subjected incident to the action of biting or chewing.

Specifically stated, the form of my invention as hereinafter described, comprises an 30 alloy having as its principal constituents, gold, platinum and palladium, with the gold predominating and the platinum forming a small proportion of the resultant metal.

My invention also includes all of the various 35 novel features as hereinafter more definitely specified.

It is commonly known that it requires heat of very high temperature to fuse or fire teeth formed of ceramic material, and that 40 the only precious metals that have been satisfactorily baked in a tooth body to form attaching means for the tooth, without fusing or otherwise disintegrating, are platinum or an alloy rich in platinum or palladium, and 45 that owing to the scarcity and consequent high cost of platinum, various means have been devised or suggested to reduce the amount of platinum or palladium employed in tooth attachments.

I have found that a metal having all of 50 the desirable characteristics of platinum for the production of pins for artificial teeth may be produced with a relatively small proportion of platinum, whereby the cost of production may be greatly reduced. 55

An alloy which produces the desirable results, contains gold, platinum and palladium, with the gold predominating to a large degree, and with the platinum forming a relatively small proportion; the gold forming about 49 per cent and the platinum forming about 14 per cent of the resultant metal.

I have found that by the introduction of a small amount of copper, the alloy formed 65 of gold, palladium and platinum may be greatly stiffened and hardened, and that an alloy which embodies the most desirable characteristics may be composed of 49 per cent gold, 37 per cent palladium, 13.45 per 70 cent platinum, and .55 per cent copper.

I do not desire to limit my invention to the precise proportions herein specified, as it is obvious that various modifications may be made therein without departing from the 75 essential features of my invention as defined in the appended claims.

Having thus described my invention, I claim:

1. An alloy containing gold, palladium 80 and platinum, in the proportions approximating 49 per cent gold, 37 per cent palladium, and 14 per cent platinum.

2. An alloy containing gold, palladium, 85 platinum and copper, in the proportions approximating 49 per cent gold, 37 per cent palladium, 13.45 per cent platinum, and .55 per cent copper.

3. An alloy of gold, palladium and platinum, with the palladium and platinum embodied in essential quantities and together 90 approximately equal to the quantity of the gold.

4. An alloy consisting of gold, palladium, platinum and copper in essential proportions 95 decreasing in the order named.

5. An alloy of gold, platinum, palladium and copper, with the palladium and plati-

num embodied in quantities together approximately equal to the quantity of the gold, and the copper forming a small proportion of the alloy but embodied in an 5 amount essential to produce a characteristic stiffness and hardness to the alloy.

In witness whereof, I have hereunto set

my hand and seal this 7th day of May, A. D., 1919.

CALVIN SPENCER VIDEON. [L. S.]

Witnesses:

W.M. H. DAVID,  
WILL R. PORTER.